

## UNITED STATES PATENT OFFICE

2,599,341

## NEW PHOSPHORUS CONTAINING COMPOUNDS

John P. McDermott, Roselle, N. J., assignor to Standard Oil Development Company, a corporation of Delaware

No Drawing. Application October 29, 1947,  
Serial No. 782,952

10 Claims. (Cl. 252—46.6)

**1**  
The present invention relates to new compounds containing phosphorus and to the uses of such compounds particularly as oxidation inhibiting additives for hydrocarbon products.

In the development of lubricating oils the trend has been to use more and more efficient refining methods in order to reduce the tendency of the oils to form carbon and deposits of solid matter or sludge. While such highly refined oils possess many advantages, their resistance to oxidation particularly under conditions of severe service is generally decreased and they are more prone to form soluble acid oxidation products which are corrosive. They are generally less effective than the untreated oils in protecting the metal surfaces which they contact against rusting and corrosion due to oxygen and moisture. They also often deposit thick films of "varnish" on hot metal surfaces, such as the pistons of internal combustion engines.

In accordance with the present invention a new class of chemical compounds has been discovered, and these compounds have been found to reduce the tendency of refined lubricating oils and other hydrocarbon products to corrode metal surfaces when added in small quantities to such materials. These additives are particularly active in reducing the corrosion of copper-lead and cadmium-silver bearings which are employed in internal combustion engines, and they are likewise effective in inhibiting the oxidation of hydrocarbon products generally and especially those of petroleum origin. These compounds also have the property of improving the load carrying capacity of mineral lubricating oils to which they are added.

The new class of compounds forming the subject of the present invention are products obtained by reacting organo-substituted acids of phosphorus, more specifically the substituted thiophosphorous, thiophosphoric, thiophosphinic, and thiophosphonic acids, or their salts, with the halides, oxyhalides and sulfohalides of phosphorus. A typical reaction is the following:



Reactions of this type take place readily without the aid of a catalyst. A suitable solvent, such as petroleum ether, is generally employed, and the halide of phosphorus is added gradually while cooling to control the reaction. It is generally more convenient to employ an alkali metal or ammonium salt of the organo-substituted acid. When an organic solvent is employed, the metallic or ammonium chloride produced in the reaction

is usually precipitated and may be removed from the product by filtration.

For purposes of nomenclature the new compounds of the present invention may be thought of as phosphorus tri- and penta-thiophosphites (di-organothiophosphites) or thiophosphates (di-organothiophosphates), when the products are formed by the reaction of phosphorus trichloride or phosphorus pentachloride with organo-substituted thiophosphites and dithiophosphates, respectively. Similarly, products derived from phosphorus oxychloride and phosphorus sulfochloride will be named phosphorus oxy tri-(di-organothiophosphites), phosphorus sulfo tri-(di-organothiophosphites), etc. Similar nomenclature will be applied to products derived from thiophosphinic and thiophosphonic acids. The products may also be thought of as anhydrides of organo-substituted acids of phosphorus. Thus 20 various compounds produced according to the method described, by selecting various combinations of organo-substituted acids of phosphorus and halides, oxyhalides or sulfohalides of phosphorus, will have compositions illustrated by the following type formulas in which R represents an organic group:



The compounds of the present invention are derived from organo-substituted acids of phosphorus, in which the organic group is a linear or cyclic hydrocarbon group, which may be straight or branched, long or short, saturated or unsaturated, and may have sulfur or halogen atoms or nitro groups attached thereto. Such organic groups will, therefore, include alkyl groups, alkenyl groups, cycloalkyl groups, and the like, with or without the substituents mentioned.

Since the organo-substituted phosphorus and phosphoric acids are usually prepared by reacting alcohols with sulfides of phosphorus it is possible

to use as starting materials a large variety of these compounds. For example, alcohols of the type of ethyl alcohol, isopropyl alcohol, tert.-butyl alcohol, lauryl alcohol, stearyl alcohol, wax alcohols, alcohols obtained by oxidation of petroleum hydrocarbons, oleyl alcohol, sulfurized oleyl alcohol, chlorinated and nitrated alcohols, cyclohexyl alcohol, and the like are suitable materials.

The phosphorus halides which are employed to react with the organo-substituted acids and their salts to form the new compounds of the present invention include all of the well known compounds of this type, such as phosphorus trichloride, phosphorus pentachloride, phosphorus oxychloride, phosphorus sulfochloride, phosphorus tribromide, phosphorus oxybromide, phosphorus triiodide, and the like, as well as mixed halides of phosphorus, such as  $\text{PCl}_2\text{F}_3$  and  $\text{PBr}_2\text{F}_3$ .

Stated broadly, the new compounds of the present invention may be defined by the general formula



in which R represents a hydrocarbon group which may or may not contain added sulfur, chlorine or nitro groups, X and Y each represent oxygen or sulfur, n, n' and n'' each represent 0 or 1, and m is 3 or 5, but is always 3 when n'' is 1.

When compounds of the above type are to be formed in which n'' is 0, or in other words when there is no free oxygen or sulfur atom attached to the phosphorus in the right hand portion of the formula, the phosphorus halides must be of the simple type, containing no oxygen or sulfur. To produce compounds in which oxygen or sulfur is present in the position Y in the formula, an oxyhalide or sulfohalide must be employed. It is to be understood that the beneficial effects of the new additives of the present invention will be obtained when mixtures of the above described types of compounds are employed in place of simple compounds, e. g., mixtures of alcohols could be employed to prepare mixed substituted acids of phosphorus and such mixed acids could then be reacted with a halide of phosphorus to obtain a mixed product, but such mixed products would be equally useful for the purposes of the present invention.

As stated above, the herein described new compounds may be advantageously added to mineral lubricating oils and other hydrocarbon products for the purpose of preventing corrosion and generally to inhibit oxidation. For this purpose, the amount of the compounds required are generally from about 0.2% to 5% by weight, relative to the base stock in which they are incorporated. For increasing the load carrying capacity of a lubricating oil to an appreciable extent, somewhat larger quantities, generally of the order of 3% to 10%, will be required.

The following examples illustrate the preparation of several examples of the new compounds of the present invention and the testing of certain of these compounds for their corrosion inhibiting effects in lubricating oils. It is to be understood, however, that these examples are not to be considered as limiting the scope of the invention in any way.

*Example 1.—Preparation of phosphorus tri-(diisopropyl dithiophosphate)*

To a stirred suspension of 115.5 g. of ammonium diisopropyl dithiophosphate in 1 liter of

petroleum ether contained in a 4-necked 3-liter flask equipped with a stirrer, reflux condenser, thermometer, and dropping funnel, was added a solution of 22.8 g. of  $\text{PCl}_3$  in 250 cc. of petroleum ether over a period of one hour (maximum temperature 25° C.). The mixture was then stirred under reflux for three hours (40–45° C.), after which the reaction mixture was permitted to stand overnight. After filtering off the ammonium chloride, the solvent was evaporated at 45° C., with nitrogen blowing. The white crystalline product contained 18.7% phosphorus and 27.9% sulfur.

*Example 2.—Preparation of phosphorus tri-(di-2-ethylhexyl dithiophosphate)*

This preparation was carried out in the manner described in Example 1, using as reagents 117.6 g. of potassium di-2-ethylhexyl dithiophosphate (prepared from the acid obtained by reacting 2-ethylhexanol with  $\text{P}_2\text{S}_5$ ) and 13.7 g. of  $\text{PCl}_3$ . The product was a clear yellow liquid containing 11.4% phosphorus and 16.4% sulfur.

*Example 3.—Preparation of phosphorus oxy-tri-(di-2-ethylhexyl dithiophosphate)*

This preparation was carried out in the manner described in Example 1, using 117.6 g. of potassium di-2-ethylhexyl dithiophosphate (prepared from the acid obtained by reacting 2-ethylhexanol with  $\text{P}_2\text{S}_5$ ) and 15.3 g. of  $\text{POCl}_3$ . The product was a clear light brown liquid containing 9.6% phosphorus and 15.4% sulfur.

*Example 4.—Preparation of phosphorus penta-(di-2-ethylhexyl dithiophosphate)*

This preparation was carried out in the manner described in Example 1, using 117.6 g. of potassium di-2-ethylhexyl dithiophosphate (prepared from the acid obtained by reacting 2-ethylhexanol with  $\text{P}_2\text{S}_5$ ) and 12.5 g. of  $\text{PCl}_3$  (suspended in 200 cc. of petroleum ether). The final product was a clear dark red liquid containing 10.3% phosphorus and 16.7% sulfur.

*Example 5.—Laboratory corrosion tests*

Lubricating oil blends were prepared containing 0.25% by weight of each of the products prepared in Examples 1 to 4, using as a base oil an extracted Mid-Continent paraffinic type lubricating oil of SAE 20 grade. These blends and a sample of the unblended oil were submitted to a corrosion test designed to measure the effectiveness of the new compounds in inhibiting the corrosiveness of a typical mineral lubricating oil toward the surfaces of copper-lead bearings. The test was conducted as follows: 500 cc. of the oil was placed in a glass oxidation tube (13 inches long and 2% inches in diameter) fitted at the bottom with a  $\frac{1}{4}$  inch air inlet tube perforated to facilitate air distribution. The oxidation tube was then immersed in a heating bath so that the oil temperature was maintained at 325° F. during the test. Two quarter sections of automotive bearings of copper-lead alloy of known weight having a total area of 25 sq. cm. were attached to opposite sides of a stainless steel rod which was then immersed in the test oil and rotated at 600 R. P. M., thus providing sufficient agitation of the sample during the test. Air was then blown through the oil at the rate of 2 cu. ft. per hour. At the end of each 4-hour period the bearings were removed, washed with naphtha and weighed to determine the amount of loss by corrosion. The bearings were then re-

polished (to increase the severity of the test), reweighed; and then subjected to the test for additional 4-hour periods in like manner. The results are given in the following table as "corrosion life," which indicates the number of hours required for the bearings to lose 100 mg. in weight, determined by interpolation of the data obtained in the various periods.

| Oil Blend                                                             | Bearing Corrosion Life (Hrs.) |
|-----------------------------------------------------------------------|-------------------------------|
| Base Oil                                                              | 9                             |
| Base Oil + 0.25% Phosphorus tri-(diisopropyl dithiophosphate)         | 52                            |
| Base Oil + 0.25% Phosphorus tri-(di-2-ethylhexyl dithiophosphate)     | 23                            |
| Base Oil + 0.25% Phosphorus oxy tri-(di-2-ethylhexyl dithiophosphate) | 19                            |
| Base Oil + 0.25% Phosphorus penta-(di-2-ethylhexyl dithiophosphate)   | 18                            |
|                                                                       | 20                            |

*Example 6.—Lauson engine test*

A blend containing 0.75% by weight of the product of Example 1 in a solvent extracted Mid-Continent paraffinic type SAE 10 grade lubricating oil base and a sample of the unblended base stock were employed as crank case lubricants in tests with a Lauson engine operated for 20 hours in each test at 300° F. jacket temperature, 295° F. oil temperature, 1800 R. P. M. speed, and 1.5 indicated kilowatt load. The effect of the additive was noted by comparing the loss in weight of the bearing during the two tests. The results are as follows:

| Oil                                                           | Cu-Pb Bearing Weight Loss (mg./bearing) |
|---------------------------------------------------------------|-----------------------------------------|
| Base Oil                                                      | 220                                     |
| Base Oil + 0.75% Phosphorus tri-(diisopropyl dithiophosphate) | 95                                      |

The products of the present invention may be employed not only in ordinary hydrocarbon lubricating oils but also in the "heavy duty" type of lubricating oils which have been compounded with such detergent type additives as metal soaps, metal petroleum sulfonates, metal phenates, metal alcoholates, metal alkyl phenol sulfides, metal organophosphates, thiophosphates, phosphites and thiophosphites, metal salicylates, metal xanthates and thioxanthates, metal thiocarbamates, amines and amine derivatives, reaction products of metal phenates and sulfur, reaction products of metal phenates and phosphorus sulfides, metal phenol sulfonates, and the like. Thus, the additives of the present invention may be used in lubricating oils containing such other addition agents as barium tert.-octylphenol sulfide, calcium tert.-amylphenol sulfide, nickel oleate, barium octadecylate, calcium phenyl stearate, zinc diisopropyl salicylate, aluminum naphthenate, calcium cetyl phosphate, barium di-tert.-amylphenol sulfide, calcium petroleum sulfonate, zinc methyl cyclohexyl thiophosphate, calcium dichloro-stearate, etc. Other types of additives, such as phenols and phenol sulfides may be employed.

The lubricating oil base stocks used in the compositions of this invention may be straight mineral lubricating oils or distillates derived from paraffinic, naphthenic, asphaltic or mixed base crudes, or, if desired, various blended oils

may be employed as well as residuals, particularly those from which asphaltic constituents have been carefully removed. The oils may be refined by conventional methods using acid, alkali and/or clay or other agents such as aluminum chloride, or they may be extracted oils produced, for example, by solvent extraction with solvents of the type of phenol, sulfur dioxide, furfural, dichloroethyl ether, nitrobenzene, crotonaldehyde, etc. Hydrogenated oils or white oils may be employed as well as synthetic oils prepared, for example, by the polymerization of olefins or by the reaction of oxides of carbon with hydrogen or by the hydrogenation of coal or its products. In certain instances cracking coal tar fractions and coal tar or shale oil distillates may also be used. Also for special applications, animal, vegetable or fish oils or their hydrogenated or volatilized products may be employed in admixture with mineral oils.

For the best results the base stock chosen should normally be that oil which without the new additive present gives the optimum performance in the service contemplated. However, since one advantage of the additives is that their use also makes feasible the employment of less satisfactory mineral oils or other oils, no strict rule can be laid down for the choice of the base stock. Certain essentials must of course be observed. The oil must possess the viscosity and volatility characteristics known to be required for the service contemplated. The oil must be a satisfactory solvent for the additive, although in some cases auxiliary solvent agents may be used. The lubricating oils, however they may have been produced, may vary considerably in viscosity and other properties depending upon the particular use for which they are desired, but they usually range from about 40 to 150 seconds Saybolt viscosity at 210° F. For the lubricating of certain low and medium speed diesel engines the general practice has often been to use a lubricating oil base stock prepared from naphthenic or aromatic crudes and having a Saybolt viscosity at 210° F. of 45 to 90 seconds and a viscosity index of 0 to 50. However, in certain types of diesel engine and other gasoline engine service, oils of higher viscosity index are often preferred, for example up to 75 to 100, or even higher, viscosity index. In addition to the materials to be added according to the present invention, other agents may also be used such as dyes, pour depressors, heat thickened fatty oils, sulfurized fatty oils, organo-metallic compounds, metallic or other soaps, sludge dispersers, antioxidants, thickeners, viscosity index improvers, oiliness agents, resins, rubber, olefin polymers, volatilized fats, volatilized mineral oils, and/or volatilized waxes and colloidal solids such as graphite or zinc oxide. Solvents and assisting agents, such as esters, ketones, alcohols, aldehydes, halogenated or nitrated compounds, and the like may also be employed.

Assisting agents which are particularly desirable as plasticizers and defoamers are the higher alcohols having eight or more carbon atoms and preferably 12 to 20 carbon atoms. The alcohols may be saturated straight and branched chain aliphatic alcohols such as octyl alcohol ( $C_8H_{17}OH$ ), lauryl alcohol, ( $C_{12}H_{25}OH$ ), cetyl alcohol ( $C_{16}H_{33}OH$ ), stearyl alcohol, sometimes referred to as octadecyl alcohol, ( $C_{18}H_{37}OH$ ), heptadecyl alcohol ( $C_{17}H_{35}OH$ ), and the like, the corresponding olefinic alcohols such as oleyl alcohol, cyclic alcohols such as naphthenic alcohols; and aryl substituted alkyl alcohols, for in-

stance, phenyl octyl alcohol, or octadecyl benzyl alcohol or mixtures of these various alcohols, which may be pure or substantially pure synthetic alcohols. One may also use mixed naturally occurring alcohols such as those found in wool fat (which is known to contain a substantial percentage of alcohols having about 16 to 18 carbon atoms) and in sperm oil (which contains a high percentage of cetyl alcohol); and although it is preferable to isolate the alcohols from those materials, for some purposes, the wool fat, sperm oil or other natural products rich in alcohols may be used per se. Products prepared synthetically by chemical processes may also be used, such as alcohols prepared by the oxydation of petroleum hydrocarbons, e. g., paraffin wax, petrolatum, etc.

In addition to being employed in crankcase lubricants the additives of the present invention may also be used in extreme pressure lubricants, engine flushing oils, industrial oils, general machinery oils, process oils, rust preventive compositions and greases.

The additives of the present invention may be employed as antioxidant or stabilizing agents not only in mineral lubricating oils, but also in hydrocarbon products generally, where improved resistance to oxidation is desired. Thus, the products may be added to motor oils, diesel fuels, kerosene, waxes, hydrocarbon polymers, natural and synthetic rubbers, etc.

The present invention is not to be considered as limited by any of the examples described herein, which are given by way of illustration only, but is to be limited solely by the terms of the appended claims.

I claim:

1. An essentially hydrocarbon oil product having incorporated therein at least a corrosion inhibiting amount of a compound of the formula 40



in which R is an alkyl group having in the range of 3 to 8 carbon atoms, X is selected from the group consisting of oxygen and sulfur, n is a number from 0 to 1, and m is an odd number from 3 to 5, but is 3 when n is 1.

2. A composition according to claim 1 in which the hydrocarbon product is a mineral lubricating oil.

3. A composition according to claim 1 in which R of the formula is an isopropyl group.

4. A composition according to claim 1 in which R of the formula is a 2-ethylhexyl group.

5. As a new composition of matter a compound of the formula



where R is an alkyl group.

6. As a new composition of matter a compound of the formula



where R is an alkyl group.

7. As a new composition of matter a compound of the formula:



8. As a new composition of matter an organic compound containing a polyvalent phosphorus atom, in which from three to five valences are satisfied by groups of the formula:



where R is an alkyl group, and in which in the case where only three valences of the phosphorus atom are thus satisfied the remaining valences are satisfied by an oxygen atom.

9. A composition according to claim 8 in which R has from 2 to 18 carbon atoms.

10. A composition according to claim 9 in which R has from 3 to 8 carbon atoms.

JOHN P. McDERMOTT.

#### REFERENCES CITED

The following references are of record in the file of this patent:

#### UNITED STATES PATENTS

| Number       | Name           | Date          |
|--------------|----------------|---------------|
| Re. 20,411   | Romieux et al. | June 15, 1937 |
| 2,038,400    | Whitworth      | Apr. 21, 1936 |
| 50 2,242,260 | Prutton        | May 20, 1941  |
| 2,336,302    | Schrader       | Dec. 7, 1943  |
| 2,343,831    | Osborne        | Mar. 7, 1944  |
| 2,514,150    | Bell           | July 4, 1950  |
| 2,526,497    | Mikeska        | Oct. 17, 1950 |